

# UNITED STATES PATENT OFFICE.

ALFRED ADAMS, JR., OF PHILADELPHIA, PENNSYLVANIA.

## FLEXIBLE-LEATHER-BOARD COMPOSITION.

1,188,600.

Specification of Letters Patent. Patented June 27, 1916.

No Drawing.

Application filed March 31, 1915. Serial No. 18,296.

*To all whom it may concern:*

Be it known that I, ALFRED ADAMS, Jr., a citizen of the United States, residing at Philadelphia, in the county of Philadelphia and State of Pennsylvania, have invented new and useful Improvements in Flexible-Leather-Board Composition, of which the following is a specification.

My invention relates to a new and useful composition of matter for producing flexible leather board to be used in the manufacture of shoes, mats, chair bottoms, upholstery and similar articles.

With these ends in view, this invention consists in the details and combination of elements hereinafter set forth and specifically designated by the claims.

In order that those skilled in the art to which this invention appertains, may understand how to make and use the same, I will describe the composition in detail.

In carrying out my invention I mix together hide and leather clippings of approximately ninety pounds, to which is added approximately ten pounds of cotton, preferably in the raw state, to provide the necessary fiber, and to these is added any suitable and well known binder, such as a mixture made of glycerin, and rubber glue, the whole mass being colored to the desired shade by adding thereto a suitable coloring pigment. These ingredients after being mixed together are beaten, shredded and stirred to produce a homogeneous mass of liquid, thin enough to flow readily, a suffi-

cient amount of the binder being added to accomplish this result. This liquid mass is then poured into molds of the desired shape and subjected to hydraulic or other high pressure, after which it is gradually dried by a slow heat to produce the flexible leather board. 40

Of course I do not wish to be limited to the exact details and combinations as herein described, as these may be varied within the limits of the appended claims without departing from the spirit of my invention. 45

Having thus fully described my invention, what I claim as new and useful, is—

1. The herein described composition of matter for producing a flexible leather board consisting of a mixture of hide and leather clippings, ninety pounds, cotton ten pounds and a liquid binder. 50

2. The herein described composition of matter for producing a flexible leather board consisting of a mixture of hide and leather clippings, ninety pounds, cotton ten pounds, and a liquid binder, the entire mixture being shredded, beaten and stirred to produce a homogeneous mass which is molded in shape, subjected to high pressure and slowly dried. 55 60

In testimony whereof, I have hereunto affixed my signature in the presence of two subscribing witnesses.

ALFRED ADAMS, JR.

Witnesses:

M. TOBIAS,  
M. P. WILLIAMSON.